

Aug. 7, 1934.

M. PIER

1,969,422

TREATMENT OF COALS, TARS, MINERAL OILS, AND THE LIKE

Filed Nov. 29, 1930

2 Sheets-Sheet 1

*Fig. 1.*



*Fig. 2.*



*Fig. 3.*



*Mathias Pier*

INVENTOR

BY *Hauff & Barland*  
ATTORNEYS

Aug. 7, 1934.

M. PIER

1,969,422

TREATMENT OF COALS, TARS, MINERAL OILS, AND THE LIKE

Filed Nov. 29, 1930

2 Sheets-Sheet 2

*Fig. 4.*



*Mathias Pier*

INVENTOR.

BY *Hauff-Strand*

ATTORNEYS.

Patented Aug. 7, 1934

1,969,422

# UNITED STATES PATENT OFFICE

1,969,422

## TREATMENT OF COALS, TARS, MINERAL OILS, AND THE LIKE

Mathias Pier, Heidelberg, Germany, assignor to Standard-I. G. Company, Linden, N. J., a corporation of Delaware

Application November 29, 1930, Serial No. 498,939  
In Germany December 3, 1929

4 Claims. (Cl. 196—133)

- The present invention relates to improvements in and materials for the treatment of coals, tars, mineral oils and the like.
- In the treatment of carbonaceous materials, such as coals of all varieties, tars, mineral oils and the like, their distillation and conversion products and residues with hydrogen or gases supplying hydrogen at elevated temperatures, if desired under pressure, and in particular in destructive hydrogenation, the inner parts of the apparatus which come into contact with the hot reacting materials are frequently strongly corroded, and the economy of the process is injuriously affected by the inconvenience in working consequent thereon. This phenomenon, which takes place mainly in the reaction chamber, but which also takes place in the adjacent hot parts such as the supply and exit pipes, the preheaters, regenerators and the like, is caused by the presence of substances which injuriously affect the material under the working conditions. These injurious substances are mainly the hydrogen and sulphur compounds arising from the initial materials combined with the action of the carbonaceous materials and of the pressure usually present. In the treatment of coals, tars, mineral oils and the like with hydrogen at elevated temperatures constructional materials must therefore be employed which are capable of withstanding the injurious influences of hydrogen and sulphur compounds in cases when the initial materials contain sulphur, as for example most kinds of coal, and crude oils, in particular crude American oil, Mexican Panuco oil, asphalts, pitches and the like.
- I have now found that the corrosion on the constructional materials of the apparatus is entirely avoided by constructing the parts, which are liable to come into contact with the hot solid, liquid or gaseous reaction materials containing sulphur, wholly or partly of a metallic material (under which expression I understand metals and alloys) which is stable or to a great extent stable to hydrogen and which is provided on the inside with a coating or lining which is insensitive to sulphur or its compounds. Alloyed steels, which contain for example from 1 to 6 per cent of chromium alone or together with other elements such as aluminium, tungsten, vanadium, cobalt, manganese, nickel and the like and which are not sufficiently resistant to sulphur may be employed for the preparation of the outer walls of the reaction vessel which are stable to hydrogen and which if desired may be pressure bearing walls, or for the preparation of other parts of the apparatus, which are not exposed to the action of sulphur or compounds thereof. Thus for example alloyed steels having the following compositions may be employed with advantage for the preparation of the outer walls:
- (1) iron containing 1 per cent of chromium, 0.2 per cent of vanadium and 0.3 per cent of carbon;
- (2) iron containing 3.8 per cent of nickel, 1.6 per cent of chromium and 0.22 per cent of carbon;
- (3) iron containing 2.5 per cent of chromium, 11 per cent of tungsten and 0.3 per cent of carbon;
- (4) iron containing 5.2 per cent of chromium, 2 per cent of nickel, 0.3 per cent of vanadium and 0.12 per cent of carbon;
- (5) iron containing 1 per cent of chromium, 1.5 per cent of manganese and 0.2 per cent of carbon;
- (6) iron containing 4 per cent of chromium, 16 per cent of tungsten, 8 per cent of cobalt, 1.5 per cent of vanadium and 0.7 per cent of carbon.
- It is to be understood, however, that the steels suitable for the purpose in question are not restricted to the examples given above but that many other combinations may also be satisfactorily employed. The inner parts of the apparatus which are exposed to the chemical attack of sulphur or compounds thereof, in particular hydrogen sulphide, organic sulphides and sulphohydrides may consist for example of silver, zinc, brass or other zinc alloys such as iron-zinc, nickel-zinc, iron-nickel-zinc, copper-iron-zinc, or also other metals such as molybdenum, tungsten, chromium, titanium, which latter metals may be applied to the inner wall of the vessel by the diffusion occurring when two metals are brought into contact with each other at high temperatures. This inner wall need not be stable to hydrogen and may consist of a thin lining or coating permeable to hydrogen, if necessary only a fraction of a millimeter in thickness. It may be applied for example electrolytically. Alloyed steels may also be provided with a coating of aluminium which has been prepared by calorizing, whereby the alloyed steel is embedded in aluminium powder and heated, or painted with aluminium bronze or sprayed with aluminium and then heated. By the same process the parts of the apparatus which come into contact with the hot reacting materials may also be provided with coatings of other metals having the same action. The walls of the vessel prepared from material which is stable to hydrogen may also be provided with coatings of a non-metal nature, as for example silicon or melts containing boron or phosphorus or boron and phosphorus in chemical combination such as boric oxide, borates, phosphates and the like, which are insensitive to the attack of sulphur at the temperature employed and which are not capable of reacting with the reacting components. In cases when the outer material stable to hydrogen is exposed to high pressures it is preferable to surround it with ordinary steel, provided if desired with de-aerating holes, to take up the pressure. The vessel and the inlet and outlet pipes and the like would then consist of an outer

65

75

80

85

90

95

100

105

110

115

120

pressure bearing wall which surrounds a wall stable to hydrogen which is provided on the inner side with a coating or lining stable to sulphur.

The apparatus according to the present invention has the great advantages that the jacket stable to hydrogen need not be prepared from material stable to sulphur which is usually expensive, and that the inner protecting layer which is stable to sulphur may be very thin since the hydrogen which diffuses through in this case is retained by the outer jacket or cannot injure it.

The nature of the invention will be further described with reference to the accompanying drawings which illustrate arrangements of apparatus according to this invention, but the invention is not restricted to these arrangements.

Figures 1, 2 and 3 shows in longitudinal section different kinds of vessels suitable for the treatment of carbonaceous materials with hydrogen at elevated temperatures according to the present invention. Figure 4 shows a plant, partly in longitudinal section, for carrying out hydrogenation according to the invention and has reference to the following Example 1.

Referring to Figure 1 numeral 1 denotes the wall of a reaction vessel which is covered with a coating 2 consisting of an iron alloy containing 6 per cent of chromium. The inner surface of this coating is provided with a further thin coating 3 consisting of silver, molybdenum, chromium or a zinc alloy.

Figure 2 shows a vessel the wall 1 of which is provided with holes 4, the walls being coated with a layer 2 consisting of an iron alloy which contains 5.2 per cent of chromium, 2 per cent of nickel, 0.3 per cent of vanadium and 0.12 per cent of carbon. The inner surface of the layer 2 is provided with a thin lining 3 of zinc or aluminium. The outer surface of the said layer is provided with a groove 5 winding spirally round it.

Figure 3 shows a reaction vessel the wall 1 of which is provided with a coating 2 consisting of an iron alloy containing 3.8 per cent of nickel, 1.6 per cent of chromium and 0.22 per cent of carbon. Between the coating 2 and the wall 1 is a free space 6 which is filled with an insulating material such as asbestos or the like, or with nitrogen or the like. When filling the said free space with a gas it is necessary that the pressure of the latter should be as great as the pressure in the reaction space. The inner surface of the coating 2 is lined with a thin layer of brass 3.

The following examples will further illustrate the nature of this invention, but the invention is not restricted to these examples.

#### Example 1

A brown coal low-temperature carbonization tar containing 1.5 per cent of sulphur is passed together with hydrogen under a pressure of 200 atmospheres at the inlet 7 shown in Figure 4 through a preheater 8 which consists of an iron alloy containing 13 per cent of chromium and 0.15 per cent of carbon and which is heated with hot gases. The materials preheated to a temperature of about 440° C. are then passed into the reaction vessel 9 where, while liquid at about 450° C., they are brought into contact with a catalyst consisting of molybdic acid and zinc oxide. The reaction vessel is lined with a coating 2 consisting of an iron alloy containing 3.3 per cent of chromium, 1.5 per cent of nickel, 0.5 per cent of manganese and 0.1 per cent of carbon. The inner surface of this coating is provided with

a layer 3 consisting of aluminium, the thickness of which is exaggerated in the drawings for the sake of clearness. The gases and vapors leaving the reaction vessel at the outlet 10 are passed through condenser 11 which consists of an iron alloy containing 3 per cent of nickel, 1.5 per cent of chromium and 0.3 per cent carbon. The inner surface of the condenser and of the preheater is also provided with a layer 3 consisting of aluminium. This layer is prepared by applying aluminium bronze to the single parts of the apparatus and then exposing them in an atmosphere of hydrogen to a temperature of about from 900° to 1000° C. In this manner a firm coating is obtained which is not substantially attacked by sulphur even after a long duration of the reaction. 15 per cent of constituents boiling to 180° C. and 60 per cent of middle oils are obtained from the initial materials.

#### Example 2

A Mexican Panuco oil containing 4.5 per cent of sulphur is brought together with hydrogen into contact with a catalyst prepared from tungstic acid, arsenic acid and manganese carbonate at 450° C. under a pressure of 200 atmospheres in a high pressure vessel. The whole of the high pressure apparatus is constructed of a material which consists of 5.3 per cent of chromium, 1.8 per cent of nickel, 0.1 per cent of carbon and the remainder iron. The parts of the apparatus which come into contact with the hot reacting materials are provided with a thin coating consisting of 60 per cent of copper and 40 per cent of zinc, which is prepared by immersing the parts of the apparatus in a liquid melt of the metals. The coating is not attacked by sulphur even after use for long periods of time. In this manner 20 per cent of constituents boiling at temperatures up to 180° C. and 60 per cent of middle oil are obtained from the initial materials.

What I claim is:—

1. An apparatus suitable for heat-treating carbonaceous materials with hydrogen, of which the parts liable to come into contact with the hot materials are composed of a base consisting of an alloyed steel containing from 1 to 6 per cent of chromium, which is internally lined with a coating of a metallic material selected from the group consisting of zinc and zinc alloys.

2. The process of destructively hydrogenating hydrocarbon products containing sulphur with hydrogen under a temperature and pressure suitable for destructive hydrogenation which comprises effecting the destructive hydrogenation in a reaction space defined by a material resistant to sulphur under the conditions of the reaction and permeable to hydrogen selected from the class consisting of zinc and alloys of zinc and preventing escape of the hydrogen from the reaction space by backing said sulphur resistant material with a hydrogen resistant hydrogen impermeable shell composed of a chromium steel.

3. The process as defined in claim 2 wherein said shell is composed of a chromium steel containing from 1 to 6 per cent of chromium.

4. The process as defined in claim 2 wherein the hydrocarbon products comprise a hydrocarbon oil containing sulphur and wherein the destructive hydrogenation is carried out at a temperature of about 450° C. and a pressure of about 200 atmospheres.

MATHIAS PIER.